

1

2,878,109

## LIQUID FUEL COMPOSITION

Joseph Francis Wood and Charles Howard Hopkins, Pawhuska, Okla., assignors to Skelly Oil Company, Tulsa, Okla., a corporation of Delaware

No Drawing. Application March 16, 1955  
Serial No. 494,807

6 Claims. (Cl. 44—58)

This invention relates to organic liquid compositions and more particularly to liquid hydrocarbons into which an additive has been incorporated.

It is known that certain liquid hydrocarbons, such as gasoline, kerosene, diesel oils, furnace oils and lubricating oils, have a tendency to form gums and gum compositions during storage under ordinary conditions. This tendency is not desirable in motor fuels, such as gasoline, diesel fuels or furnace oils, since the gums or gumlike substances may result in valve and line clogging in carburetors and other fuel-feeding or fuel induction systems or the formation of deposits in the combustion zone. Also upon storage of products of this general character the hydrocarbon compositions have a tendency to accumulate small amounts of water due, at least in part, to condensation from the atmosphere. Such water interferes with the use of the composition as a fuel or lubricant and may also give rise to corrosion problems. In the past, various additives have been proposed to combat the gum problem but these compounds are generally of the nature of detergents which, in so far as they may be effective, act to prevent the accumulation of gum in various types of equipment in which the hydrocarbon liquid is employed, the detergents merely preventing the accumulation of gum or gumlike materials. In so far as the water problem is concerned, the additives that have been employed for this purpose are generally corrosion inhibitors and freezing point depressants. However, they are generally not effective for removing the water from the hydrocarbon liquid.

Accordingly, an object of this invention is the provision of a liquid hydrocarbon composition having contained therein an additive which prevents the formation of gums, lacquers, varnishes and similar materials in the fuel induction systems and combustion zones in which the hydrocarbon may be used.

A further object of the invention is the provision of an additive for a hydrocarbon which prevents the accumulation of water therein even upon storage thereby providing a gasoline, kerosene, diesel fuel, furnace oil, lubricating oil or other heavy liquid petroleum product which is essentially anhydrous at all times.

A further object of this invention is the provision of a motor fuel which modifies or eliminates combustion chamber deposits when employed so that such deposits do not change the operating conditions of the engine.

A still further object of this invention is the provision of an additive for a motor fuel which improves the volatility thereof without giving rise to detrimental vapor lock effects, thereby improving the starting characteristics of the fuel.

A further object of this invention is the provision of an additive for gasoline or other motor fuel which has a research octane blending value in excess of 100.

A further object of this invention is the provision of an additive for a gasoline which raises the practical limit of compression in spark ignition engines.

2

A still further object of this invention is the provision of an additive for a motor fuel which retards compression-excited pre-ignition.

A further object of this invention is the provision of a hydrocarbon composition which remains essentially free of water, thereby eliminating the formation of rust or problems incident to freezing in storage and induction systems.

A further object of this invention is the provision of a motor fuel in which the exhaust gas odors have been diminished.

A further object of this invention is the provision of a hydrocarbon composition of increased stability against oxidation.

A still further object of this invention is the provision of a hydrocarbon product providing increased spark plug life and valve life through the removal or minimizing of gumlike deposits.

A still further object of this invention is the provision of a furnace oil which is stabilized against gum formation and the accumulation of water therein.

Further and additional objects will appear from the following description and the accompanying claims.

In accordance with this invention, a liquid hydrocarbon or other organic liquid is treated with a ketal in order to provide a composition having one or more of the above indicated desirable characteristics. The ketal employed in accordance with this invention is 2,2-dimethoxypropane. The ketal reacts with water to produce one molecule of an acetone and two molecules of a methanol with the consequent consumption of one molecule of water. The ketal, as well as the ketone and alcohol, serves as a solvent which tends to prevent the formation of gum, lacquers, varnishes or the like during storage of the hydrocarbon or when the hydrocarbon may be burned in an internal combustion engine. The ketal employed as an additive in accordance with the disclosure of this invention is to be sharply distinguished from those compounds which are specifically known as acetals and which are the condensation products of two mols of an alcohol with one mol of an aldehyde. Thus if acetals are employed as additives for a hydrocarbon, they will react with accumulated water to form an alcohol and an aldehyde. Such aldehydes are wholly undesirable in hydrocarbon liquids since the aldehydes themselves tend to undergo polymerization thereby producing gummylike materials and resinous products which are avoided in the products of this invention.

In accordance with one embodiment of this invention, it is preferred to add to the hydrocarbon liquid, in addition to the ketal, a substance which will catalyze the reaction between water and the ketal, thereby insuring prompt removal of any accumulated water as such from the hydrocarbon liquid. Such catalysts are generally acidic in nature and are preferably those organic compounds which are soluble in the liquid hydrocarbon and which may be readily hydrolyzed to form an acid. Specific compounds of this nature are the hydrochlorides of the following organic nitrogenous bases:

|    |                    |                 |
|----|--------------------|-----------------|
| 60 | Aminophenol        | Phenylhydrazine |
|    | Aniline            | Picoline        |
|    | Anisidine          | Piperidine      |
|    | Iso-quinoline      | Pyridine        |
|    | Lutidine           | Pyrrolidine     |
| 65 | N-methyl aniline   | Quinoline       |
|    | N-methyl toluidine | Toluidine       |
|    | N-methyl xylidine  | Xylidine        |
|    |                    | Phenetidine     |

70 However, it will be apparent that other acid salts of the above-mentioned or other organic nitrogenous bases may be employed for this purpose if desired. Thus the hy-

drochlorides or the corresponding iodides, bromides, nitrates, nitrites, sulfates, sulfites, phosphates, phosphites, perchlorates or suitable organic acid salts of any suitable aliphatic, aromatic, homocyclic or heterocyclic organic nitrogenous compound may be employed. While it might in some instances be possible to use an acid per se as the catalyst, this is not generally advisable because of corrosion problems that may result. The salts indicated above give an acid reaction to the water which has accumulated but when the water has all reacted, the salts reform and are not essentially acidic in nature.

The amount of ketal to be added to the hydrocarbon liquid will depend in a large measure upon the character of the liquid; the purpose for which it is to be used, and the expected storage conditions. Generally speaking, the amount of ketal employed is between about 0.005 and 4.0 volume percent of the hydrocarbon. Preferably, however, the amounts will range between 0.01 and 2.0 percent by volume. Such amounts have been found to be wholly effective for the treatment of gasoline, furnace oil and lubricating oil compositions. However, it is conceivable that in certain special instances, such as in the formulation of jet engine fuels, percentages of ketal higher than indicated above could be employed to advantage.

The amount of catalytic material incorporated into the hydrocarbon mixture to assist in the hydrolytic reaction is very small and the concentration will, of course, be dependent in part upon the specific catalytic activity of the catalyst in the presence of any small amount of accumulated water. Generally speaking, it may be stated that such amounts of catalyst are usually less than one percent by weight of the ketal present and suitably between about 0.001 and 1.0 percent by weight of the ketal present in the final composition.

For a more complete understanding of this invention, reference will now be made to certain examples and test results which have been carried out demonstrating the advantages that may be obtained by adding a ketal to a hydrocarbon liquid as previously suggested.

#### Example 1

A gasoline composition was prepared admixing 1.8 cc. of 2,2-dimethoxypropane to each gallon of a conventional leaded gasoline, the concentration of ketal in the final product being 0.0475 volume percent. The ketal was thoroughly dispersed in the gasoline since it is completely miscible therein in the proportions employed. The resulting fuel was employed in a spark-ignited, water-cooled internal combustion engine which had previously been intentionally fouled with gum, varnish, lacquer and carbonaceous deposits in the fuel system and in the combustion chamber to a point wherein starting of the engine was exceedingly difficult and uniform operation was impossible to maintain. After 4 hours' operation of the engine on the ketal-hydrocarbon fuel blend, the engine started with ease, operated at constant speed without continual adjustments, and the operation of the engine was generally smooth. At the end of 40 hours' operation on the ketal-hydrocarbon fuel blend, the engine was examined revealing the removal of all gum, varnish and lacquer from the fuel storage and induction system, a total absence of accumulated water in the fuel tank and fuel strainer, and a substantial reduction in the amount of carbonaceous material in the combustion chamber on the intake and exhaust valves and on the spark plug electrode. Deposits remaining in the combustion chamber were examined and compared to original deposit samples and were found to be more porous, not as hard, and less adherent to the exposed metal with a tendency to flake off.

#### Example 2

A modern 1954 model automobile was chosen having a high compression engine which had a characteristic such that after engine deposits had accumulated during

a period of operation the best commercial gasolines no longer satisfied the octane requirements of the engine by the manufacturer's recommended basic spark setting. This particular car model is representative of a large number of cars now being manufactured. The first step was to drive the car until the engine deposits had stabilized and the octane requirement leveled off. A standard commercial leaded gasoline having a research method octane rating of 92.4 was used during the preliminary stabilization period. After about 6,000 miles, frequent octane requirement tests were made to determine the car octane demand. At this point the octane requirement was constant at a reference fuel octane number of 95.5. At 7,912 miles the car engine was disassembled for inspection. Considerable gum was found to be present in the carburetor and the amount of combustion chamber deposit on the pistons, valves, block and head was observed, but the deposits were not disturbed. The engine was then reassembled.

After reassembly of the engine, the use of a gasoline containing 1.8 cc. of 2,2-dimethoxypropane per gallon was begun. The gasoline was the same as used initially except for the addition of the ketal. After 1,000 miles of town driving using the gasoline containing ketal, the octane requirement of the engine had decreased to a reference fuel octane number of 92.0. Another 2,000 miles of similar driving indicated that the octane requirement had leveled off at 92.0. This test, therefore, indicated that the use of the ketal lowered the octane requirement of this car from 95.5 to 92.0, or about 3.5 reference fuel octane numbers.

In this same test and before the ketal was added to the fuel, the car road-rated the commercial fuel from 1.5 to 2.5 octane numbers below the ASTM-CFR research octane number for that fuel. After the ketal was added to the commercial fuel, the road rating for this fuel was from 0.5 octane number less to 1.0 octane number higher than the research octane rating, thereby demonstrating an improvement in the road octane rating of the commercial fuel when the ketal was added. Other improvements in performance characteristics of the engine were noted.

#### Example 3

The engine performance improvement and elimination of carbon deposits noted in the foregoing examples are due to the presence of the ketal in the fuel when burned. In a situation where the fuel is to be subjected to storage with a tendency to accumulate water by condensation from the atmosphere or otherwise, it is desirable to use the readily hydrolyzable catalyst to insure that the hydrolytic reaction will occur readily. Thus a fuel which will remain anhydrous during normal storage conditions including storage in an automobile gasoline tank is one in which about 2 cc. of 2,2-dimethoxypropane have been added to each gallon of gasoline and into which has been incorporated about 0.05 percent (based upon the weight of the ketal) of aniline hydrochloride or pyridine hydrochloride. In such a fuel water accumulation is prevented and the acetone and methyl alcohol formed by hydrolysis also contribute to the desirable performance characteristics of the motor fuel noted above.

#### Example 4

A No. 2 furnace oil was treated with 4.0 cc. per gallon (0.11 volume percent) of 2,2-dimethoxypropane and 0.1 percent (based on the weight of the ketal) of pyridine hydrochloride and subjected to storage. The furnace oil thus treated remained free from water during ordinary storage conditions and showed a marked decrease in the tendency toward gum formation, thereby rendering the oil more suitable for use in oil burners with a decreased tendency to clog the lines, valves and nozzles of the fuel induction system.

In the foregoing, specific examples have been given

relative to gasolines and furnace oils that may contain additives in accordance with this invention. It will, however, be apparent that other specific procedures, variations and formulations may be employed without departing from the spirit and scope of this invention. For example, in one instance it has been possible to eliminate acceleration knock, erratic cold starting and performance of an engine by the addition of 500 cc. of dimethoxypropane to 15 gallons of gasoline contained in the gasoline tank. The improvement was audibly noticeable almost instantly (less than 10 miles' operation) and the improved engine operation was evident at the first cold start.

While the invention has been specifically described with respect to the treatment of gasoline and furnace oils, it will also be apparent that it has broader applicability in connection with jet fuels, kerosenes, lubricating oils and other organic liquid treatment wherein water accumulation or gum formation may present a problem. For example, it has been found that the ketal is of use in connection with the treatment of detergent and nondetergent lube oils from which it is possible to eliminate the water or to prevent the accumulation thereof. The accumulation of water is a serious problem in automotive engine lubrication particularly where hydraulic valve lifters are employed. By eliminating the water, corrosive damage to the valve lifters and other engine parts is minimized if not eliminated in most cases.

Another field of application of this invention resides in the elimination of the effects of water corrosion in crude oil primary processing. Thus in instances where the presence of water is undesirable a ketal as above defined and a readily hydrolyzable salt may be added to the oil in order to remove water or to prevent its accumulation prior to processing.

An important feature of this invention is that the ketal additive is not incompatible with other additives that may be employed in the hydrocarbon liquid. Thus the gasolines or other oils may contain other additives such as lead tetraethyl, organic phosphates, detergents, alco-

hols or glycols without adversely affecting the intended use of the composition.

While several particular embodiments of this invention are shown above, it will be understood, of course, that the invention is not to be limited thereto, since many modifications may be made, and it is contemplated, therefore, by the appended claims, to cover any such modifications as fall within the true spirit and scope of this invention.

10 We claim:

1. A liquid hydrocarbon fuel having dispersed therein between about 0.01 and about 2.0 volume percent of 2,2-dimethoxypropane.
2. A liquid hydrocarbon fuel having added thereto between about 0.005 and about 4 percent by volume of 2,2-dimethoxypropane.
3. A gasoline motor fuel having dispersed therein between about 0.005 and about 4.0 volume percent of 2,2-dimethoxypropane.
4. A gasoline motor fuel having dispersed therein between about 0.01 and 2.0 volume percent of 2,2-dimethoxypropane.
5. A leaded gasoline containing about 0.0475 volume percent of 2,2-dimethoxypropane.
- 25 6. The product of claim 2 wherein said fuel is a furnace oil.

#### References Cited in the file of this patent

##### UNITED STATES PATENTS

|    |           |                |       |               |
|----|-----------|----------------|-------|---------------|
| 30 | 1,570,059 | Hammond        | ----- | Jan. 19, 1926 |
|    | 1,582,420 | Nikaido        | ----- | Apr. 27, 1926 |
|    | 2,106,662 | Savage         | ----- | Jan. 25, 1938 |
|    | 2,143,870 | Ellis          | ----- | Jan. 17, 1939 |
| 35 | 2,312,790 | Backoff et al. | ----- | Mar. 2, 1943  |
|    | 2,473,994 | Gresham        | ----- | June 21, 1949 |
|    | 2,626,209 | Morrell        | ----- | Jan. 20, 1953 |

##### FOREIGN PATENTS

|    |         |               |       |               |
|----|---------|---------------|-------|---------------|
| 40 | 668,664 | Great Britain | ----- | Mar. 19, 1952 |
|----|---------|---------------|-------|---------------|